

Aug. 8, 1939.

G. W. WARDWELL, JR

2,169,118

COATING FOR HEATED SURFACES

Filed Nov. 25, 1936



Fig. 2.



Inventor:  
George W. Wardwell, Jr.,  
by Harry C. Dunham  
His Attorney.

## UNITED STATES PATENT OFFICE

2,169,118

## COATING FOR HEATED SURFACES

George W. Wardwell, Jr., Nichols, Conn., assignor to General Electric Company, a corporation of New York

Application November 25, 1936, Serial No. 112,739

3. Claims. (Cl. 38—66)

The present invention relates to a protective coating for heated surfaces, which decreases the danger of burning due to accidental contact therewith.

5 The object of my invention is to provide an improved coating of this nature.

In the accompanying drawing, Fig. 1 is an end elevation of an ironing press equipped with a shoe embodying my invention, and Fig. 2 is an 10 enlarged fragmentary sectional view of the shoe.

The coating embodying my invention is particularly adapted for coating the housings or outer casings of electrically heated appliances such as ironers, waffle irons, toasters, hair dryers, 15 etc. Irons, for example, are operated at temperatures of from 250° F. to 450° F., and the outer casing will therefore normally be at a high enough temperature to cause burning or at least some discomfort upon accidental contact therewith.

20 For the purpose of illustration, I have shown my invention applied to an ironing press of the type shown in my application Serial No. 750,620 filed Oct. 30, 1934, which has matured into Patent No. 2,135,266, granted Nov. 1, 1938.

25 In this construction the pressure developing mechanism is contained within a cylinder 1 having a flange 2 for supporting the cylinder on the top 3 of a suitable table. Within the cylinder is a piston at the top of which is mounted a 30 suitably padded buck 4. On the lower end of the cylinder is pivoted a carriage 5 having an arm 6 which supports a heated shoe 7. The shoe is moved into and out of register of the buck by means of handle 8 attached to the front end 35 of the shoe. The rearward movement of the carriage is limited by a spring 9 connected to toggle links 10 and 11 which are respectively pivoted to the cylinder and to the carriage.

The construction of the shoe is shown in detail 40 in Fig. 2. The shoe comprises a metal casting 12 preferably of a material having good heat conductivity, such as aluminum. The shoe is heated by an electric heating element 13 enclosed in a metal sheath 14 which is held in a groove 15 in the upper face of the casting 12 by means of clamps 16. The lower face 17 of the casting 12 serves as the work contacting surface. The upper face of the casting 12 is enclosed by a sheet metal cover 18 which is suitably attached thereto in a manner not shown. Since the cover is spaced 45 from the casting 12 its temperature is somewhat less than the temperature of the casting which ranges from 250 to 450° F. Its temperature is, however, usually high enough to cause some discomfort and possibly even burning of the operators' hand in case of accidental contact therewith. In order to eliminate this danger, I have 50 provided a suede-like coating on the outer sur-

face of the cover which comprises short fibers or flock 19 held on the cover by a coating of a suitable cement 20, such as a varnish. The flock may comprise any suitable fibers, for example finely ground cotton. The coating may be applied by first coating the cover with the varnish and blowing the flock by means of compressed air against the varnish before it has dried. This provides a coating in which the inner ends of the fibers are embedded in the varnish 5 and the outer ends of the fibers project outwardly away from the varnish. The arrangement of the fibers will, of course, not be uniform as shown in Fig. 2, but a large number of the fibers will project substantially perpendicularly from the varnish film as illustrated. I find that this coating eliminates all danger of burning or discomfort caused by accidental contact with the shoe cover. This is not due to the heat insulating properties 10 of the flock but is rather due to the fact that the flock prevents good contact between the operator's hand and the shoe cover, thus decreasing the rate of heat transfer.

15 What I claim as new and desire to secure by Letters Patent of the United States is:

20 1. In an ironer, a shoe comprising a heated metallic body having a work engaging face and having a metal cover enclosing the opposite face, and a suede-like coating on the outside of said cover comprising flock held thereon by a cement, 25 said coating being relatively thin so as not to be substantially heat insulating and having a large number of fibers projecting from said cement so as to minimize burning or discomfort upon accidental contact therewith.

25 2. In a heating appliance, a heating means therefor, a metallic enclosure, and a coating covering the outside of said enclosure comprising flock held thereon by a cement, said coating being relatively thin so as not to be substantially 30 heat insulating and having a large number of fibers projecting from said cement so as to minimize burning or discomfort upon accidental contact therewith.

30 3. In a heating appliance, a heating means 35 therefor and a cooperating metallic member which is heated during operation of the appliance to a temperature which would cause burning or discomfort to an operator upon accidental contact therewith, and a coating covering the 40 surface of said metallic member comprising flock held thereon by a cement, said coating being relatively thin so as not to be substantially heat insulating and having a large number of fibers 45 projecting from said cement so as to minimize burning or discomfort upon accidental contact therewith.

GEORGE W. WARDWELL, JR.